

93

Cross Reference  
H. C. GOODELL.  
BOILER COVERING.

No. 274,933.

Patented Apr. 3, 1883.



Attest:

Walter Donaldson  
F. L. Middleton

Henry C. Goodell  
Inventor  
by  
Eric Spear  
Atty.

106

93

274,933

UNITED STATES PATENT OFFICE.

HENRY C. GOODELL, OF ATCHISON, KANSAS.

BOILER-COVERING.

SPECIFICATION forming part of Letters Patent No. 274,933, dated April 3, 1883.

Application filed April 7, 1882. Renewed February 24, 1883. (No model.)

To all whom it may concern:

Be it known that I, HENRY C. GOODELL, of Atchison, in the county of Atchison and State of Kansas, have invented a new and useful Improvement in Boiler-Coverings; and I do hereby declare that the following is a full, clear, and exact description of the same.

My invention relates to the covering of pipes, boilers, and like structures in which the heat producing or conveying medium is held or conveyed; and my object is to provide an economical covering which shall at the same time be an effective means for preventing the escape and consequent loss of heat by surface radiation or contact with other bodies, and shall also be easily applied.

My invention consists, essentially, of a plastic compound composed of lamp-black with a fibrous or plastic material, or either of them, mixed therewith, and adapted to be applied and to harden upon the surface of the pipe, boiler, or other structure from or into which the passage of the heat is to be obstructed.

Hereinafter I have fully described my invention and the best means known to me for the practical use and application of it.

In the accompanying drawing the figure shows a section of a boiler with my improved covering applied to its surface.

In Letters Patent of the United States reissued on the 30th day of November, 1880, and numbered 9,483, is described a receptacle provided with double walls, with a filling of lamp-black to render the walls, as far as practicable, impervious to the passage of caloric. The loose lamp-black—that is to say, lamp-black in its ordinary condition, unmixed, or with a percentage of fibrous material—is a non-conductor of heat when placed between double walls; but it is not practicable so to apply the material upon pipes which are used to convey steam, hot air, or for like purposes, nor upon the outside shells of boilers or other heat-generators. Nor is it practicable to apply the lamp-black mixed with cement or lime alone directly to the surfaces, by reason of the lack of adhesiveness of the mixture. Further, in order to give the best results, certain details of construction are essential or important, consisting in applying the coating in two or more layers. These are shown in the accompany-

ing drawing, in which is represented a section of part of a boiler-shell coated in accordance with my invention.

In carrying out my invention, when applying it to the coating of smooth boilers, pipes, or like surfaces, I coat said surfaces with a mixture to which, when applied, the mixture containing the lamp-black will adhere. This first coat consists of seventy parts well-slaked quicklime, thirty parts of crushed or ground asbestos, and enough of water to make a thick mortar. The amount of asbestos may be increased under some circumstances to give sufficient adhesiveness. Some lamp-black may be added to this first coat, if necessary. This coating is applied directly to the pipe or other surface, said surface being preferably hot when so covered, as the asbestos sticks more readily to the heated surface. For a second coating I take of well-slaked quicklime fifty parts, of vegetable coarse fiber thirty parts, and of china-clay twenty parts. These ingredients I mix with water and bring to a proper temper, and afterward add to them of lamp-black from thirty to fifty parts. The difficulty of penetrating lamp-black with water makes it necessary to first mix the other ingredients and then to add the lamp-black thereto. The body of the covering—that is to say, the largest proportion of it—is of this second composition just described. This, notwithstanding the large proportion of the lamp-black, which is not in itself adhesive, will stick to the rough coating first applied, and it may be put on in any desired thickness corresponding to the degree of heat to be resisted. It is not necessary to mix the asbestos fiber with this second coating, as it will not ordinarily be subjected to sufficient heat to destroy the vegetable fiber. Hair might be used, but not so well, as it is liable to lose its strength under the heat. The second coating is put on with a trowel or some equivalent instrument, and when it is sufficiently dry I prefer to wrap it with well-annealed wire, in circumstances where it can be done. This renders the coating solid and permanent. For the under side of large surfaces it might be necessary to apply the wire before the second coating was all on—that is to say, after the first layer of it was put on—as it may be applied in several layers. This would prevent sagging of the

heavy body of coating. After the second coating is applied, for a finish I may add a third coating, consisting of well-slaked quicklime, twenty parts; finely-ground fiber, ten parts; china-clay, fifty parts, thoroughly mixed with water, with twenty-five to thirty-five parts of lamp-black subsequently added.

Though I have specified particularly the parts, it will be understood that these proportions are not necessarily to be adhered to closely; but there may be variations within considerable limits without material variation in the result. I have specified what I consider the best proportions. On a large oval surface, for example, much greater proportion of lamp-black can be used than on a small oval surface. It will be apparent that in many cases much greater amount of adhesiveness will be required than in others, and the coatings may be varied accordingly. Under no circumstances need exactness or nicety be used in mixing the parts.

Under some circumstances the third coating may be omitted where the first and second would give sufficient protection and finish.

Instead of the lime, I may use cement, plaster-of-paris, or any equivalents of these substances. For the vegetable fiber I may use wood and paper pulp or the fiber of other vegetable substances.

It is better to apply the mixture of asbestos and lime to the surface of the iron in small quantities, like patchwork, at first, instead of spreading it all on at once, like ordinary mortar. On very rough boilers this first coating might not be necessary. I have found that a coating such as I have described from three-fourths of an inch to an inch and a quarter gives excellent results.

In the drawing I have represented the iron at *a*, the first coating at *b*, and the second coating at *c*. The wire coating is indicated at *d*, and the outer or finishing coat at *f*.

It will be apparent that these coatings may be applied to steam-boilers, steam and hot-air

pipes, or any similar pipes or vessels. It is, in fact, applicable to any situation where the passage of heat is to be prevented, and would serve as a desirable plaster and roof-covering for houses in hot climates.

50

I am aware that it has heretofore been proposed to mix soot, bone-dust, ground charcoal, and carbonaceous matter generally, with oil and argillaceous earth, and also to mix soot-ashes, rye-flour, hydraulic cement, flaxseed-meal, hair, and water for coverings for steam-boilers; and I am aware that asbestos has been mixed with plastic material in such coverings, and I do not broadly claim either carbonaceous material or asbestos in such mixtures for the covering of pipes and boilers.

55

I claim—

1. As a covering for boilers and like surfaces, a mixture consisting of the following ingredients, in substantially the proportions specified, viz: lime, fifty parts; vegetable fiber, thirty parts; china-clay, twenty parts; and of lamp-black, from thirty to fifty parts.

60

2. In a covering of boilers and the like, a layer composed of quicklime, vegetable fiber, china-clay, and lamp-black.

70

3. A finishing-coat for boilers and the like, consisting of quicklime, twenty parts; finely-ground vegetable fiber, twenty parts; china-clay, fifty parts; and of lamp-black, from twenty-five to thirty-five parts.

75

4. A covering for boilers and like surfaces, consisting of a layer of plastic material mixed with asbestos, and an outer coating of plastic material mixed with vegetable fiber and lamp-black, in substantially the proportions specified.

80

In testimony whereof I have signed my name to this specification in the presence of two subscribing witnesses.

HENRY C. GOODELL.

Witnesses:

G. E. SCOVILLE,  
RAY C. CRAWFORD.